

June 24, 1930.

L. LISSE

1,767,182

BLASTING CARTRIDGE WITH COVER AND PROCESS OF PRODUCTION

Filed March 14, 1929



Fig.1.



Fig.2.



Fig.3.

Inventor.

Dr Leopold Lisse

## UNITED STATES PATENT OFFICE

LEOPOLD LISSE, OF BERLIN-LICHTERFELDE, GERMANY

## BLASTING CARTRIDGE WITH COVER AND PROCESS OF PRODUCTION

Application filed March 14, 1929, Serial No. 347,141, and in Germany January 12, 1928.

This invention relates to a covering sleeve for cartridges and to a method for producing the covering sleeve on the cartridge so that one and the same cartridge can be used for the most various effects in using for instance a cover possessing dynamic effect increasing the dynamic effect of the blasting cartridge or, for reducing the dynamic effect of the cartridge, a cover is used which has a less great or no explosive effect, said cover covering the cartridge entirely or partly.

The novelty of the invention consists in that, after saturation of the cartridge, the impregnated and saturated cartridge is enveloped in a sheet of aluminium foil or in an envelope having a similar effect in order to increase or decrease the dynamic effect of the cartridge, so that according to requirement a dynamic explosive effect can be obtained with a less explosive cartridge than with a cartridge, which is explosive itself, a less strong dynamic effect can be obtained according to whether the cartridge is enveloped completely or partly. Instead of wrapping the impregnated cartridge in aluminium foil or in a foil of a similar metal or substitute metal, it may be rolled in metal powder and thus covered entirely or partly with the metal. A cartridge possessing dynamic effect may be transformed into a safety cartridge by enclosing it, after the impregnation, in water-containing or flame extinguishing means.

By this new process the great economic advantage is obtained that, in mines or at other places where cartridges with different dynamic effects are required, only one kind of cartridges need be kept in store. The cartridge is then, according to requirement, prepared for stronger dynamic effect or as safety cartridge, before it is used after the saturation.

It is consequently impossible that mistakes in selecting cartridges be made, as only cartridges of the same composition are used for the different purposes.

Instead of covering or coating the cartridge, the bore hole might be lined with the

suitable material into which the cartridge is then inserted.

Two embodiments of the invention are illustrated by way of example, in the accompanying drawing;

Fig. 1 shows a cartridge in elevation and the enclosing sleeve in section.

Fig. 2 shows in section a cartridge and its enclosing sleeve of another form of construction than shown in Fig. 1.

Fig. 3 is a cross section of Fig. 1.

The sleeve *a* is placed over the cartridge envelope *b* which holds the explosive material *c*. The sleeve *a* is made of fire proof material or of fire extinguishing material and rendered fire-proof or incombustible with or without a matrix. This can be done by dipping the sleeve *a* into a mixture of infusorial silica, salt or similar water-containing or incombustible material so that it is impregnated, or by coating it with such a substance with the aid of a matrix, like waterglass. For higher dynamic effect the cartridge, consisting of the charge *d* and of an envelope *e*, may, after having been saturated, be enclosed entirely or partly with an aluminium foil *f* or with a sleeve of a material having a similar dynamic effect, the cartridge being then fired. Instead of wrapping the cartridge after saturation in a metal foil, it might be rolled in a metal powder.

It has become known to add to blasting cartridges aluminium powder and similar metal powders for increasing the explosion temperature, the consumers have however complained of the inconvenience that they have to keep in store in one mine two different kinds of cartridges if, in the interest of the work to be done, blasting cartridges of different dynamic powers have to be used.

Experiments have shown that a blasting cartridge of medium dynamic effect, after having been impregnated with liquid oxygen, is transformed, between the removing of the cartridge from the impregnating vessel and the introduction into the bore hole or the placing on the object to be blasted, into a blasting cartridge possessing dynamic

55

60

65

70

75

80

85

90

95

100

effect, by rolling the moist or freshly impregnated blasting cartridge over a sheet of aluminium foil so that this foil adheres on the entire length of the cartridge, the cartridge being then inserted into the bore hole with this cover.

5 A similar result can be obtained by producing on the blasting cartridge, saturated with liquid oxygen, a coating by rolling the cartridge after the impregnation in aluminium powder or in any other suitable powder.

I claim:—

1. A process of regulating the dynamic 15 effect of blasting cartridges, consisting in covering the cartridge coming from the impregnating bath with aluminium or equivalent material, said coating being of a thickness according to the degree of dynamic 20 effect to be obtained.

2. A process of regulating the dynamic effect of blasting cartridges impregnated with liquefied gas, consisting in covering the cartridge after the impregnation with a 25 coating whereby the evaporation of the liquid is regulated.

In testimony whereof I affix my signature.

DR. LEOPOLD LISSE.

30

35

40

45

50

55

60

65